

## [54] CORONA GENERATING DEVICE

[75] Inventor: Louis Reale, Rochester, N.Y.

[73] Assignee: Xerox Corporation, Stamford, Conn.

[21] Appl. No.: 328,844

[22] Filed: Mar. 27, 1989

[51] Int. Cl. 5 H01T 19/00

[52] U.S. Cl. 250/324, 250/326;  
361/230[58] Field of Search 250/324, 325, 326;  
361/230, 225; 346/155, 150; 155/3 CH

## [56] References Cited

## U.S. PATENT DOCUMENTS

- |           |         |                 |       |          |
|-----------|---------|-----------------|-------|----------|
| 2,836,725 | 5/1958  | Uyverberg       | ..... | 250/49.5 |
| 4,086,650 | 4/1978  | Davis et al.    | ..... | 361/229  |
| 4,265,990 | 5/1981  | Stolka et al.   | ..... | 430/59   |
| 4,585,320 | 4/1986  | Altavela et al. | ..... | 355/3 CH |
| 4,585,322 | 4/1986  | Reale           | ..... | 355/3 CH |
| 4,585,323 | 4/1986  | Ewing et al.    | ..... | 355/3 CH |
| 4,646,196 | 2/1987  | Reale           | ..... | 361/230  |
| 4,792,680 | 12/1988 | Lang et al.     | ..... | 361/230  |
| 4,837,658 | 6/1989  | Reale           | ..... | 361/230  |
| 4,853,719 | 8/1989  | Reale           | ..... | 346/150  |

## OTHER PUBLICATIONS

Research Disclosure Journal, Item No. 19957, dated Nov. 1980, at p. 508, titled "Corona Discharge Unit".

Primary Examiner—Bruce C. Anderson

[57]

## ABSTRACT

A corona generating device for depositing negative charge on the imaging surface carried on a conductive substrate comprises at least one elongated conductive corona discharge electrode, means to connect the electrode to a corona generating potential source, at least one element adjacent the corona discharge electrode capable of adsorbing nitrogen oxide species generated when the electrode is energized and capable of desorbing nitrogen oxide species once that electrode is not energized, the element being coated with a substantially continuous thin conductive dry film of aluminum hydroxide containing graphite and powdered nickel. In a preferred embodiment, the conductive corona discharge electrode comprises a scorotron with at least one linear array of pin coronodes where the corona control grid is coated with the film.

17 Claims, 5 Drawing Sheets



FIG. 1





FIG. 3



FIG. 4



FIG. 5



## CORONA GENERATING DEVICE

## REFERENCE TO RELATED APPLICATIONS

Reference is hereby made to my copending applications U.S. Ser. No. 284,225 entitled "Coated Ion Projection Printing Head" filed currently herewith and U.S. Ser. No. 284,224 entitled "Long life Corona Charging Device" also filed both Dec. 14, 1988.

Reference is also made to copending application Ser. No. 002,100 entitled "Corona Device Having a Beryllium Copper Screen" filed Jan. 12, 1987 in the name of Lang et al.

## BACKGROUND OF THE INVENTION

The present invention relates generally to charging devices and in particular to charging devices which produce a negative corona.

In an electrostatographic reproducing apparatus commonly used today, a photoconductive insulating member may be charged to a negative potential, thereafter exposed to a light image of an original document to be reproduced. The exposure discharges the photoconductive insulating surface in exposed or background areas and creates an electrostatic latent image on the member which corresponds to the image areas contained within the original document. Subsequently, the electrostatic latent image on the photoconductive insulating surface is made visible by developing the image with a developing powder referred to in the art as toner. During development the toner particles are attracted from the carrier particles by the charge pattern of the image areas on the photoconductive insulating area to form a powder image on the photoconductive area. This image may be subsequently transferred to a support surface such as copy paper to which it may be permanently affixed by heating or by the application of pressure. Following transfer of the toner image to the support surface the photoconductive insulating surface may be discharged and cleaned of residual toner to prepare for the next imaging cycle.

Various types of charging devices have been used to charge or precharge photoconductive insulating layers. In commercial use, for example, are various types of corona generating devices to which a high voltage of 45 5,000 to 8,000 volts may be applied to the corotron device thereby producing a corona spray which imparts electrostatic charge to the surface of the photoreceptor. One particular device would take the form of a single corona wire strung between insulating end blocks 50 mounted on either end of a channel or shield. Another device, which is frequently used to provide more uniform charging and to prevent overcharging, is a scorotron which comprises two or more corona wires with a control grid or screen of parallel wires or apertures in a 55 plate positioned between the corona wires and the photoconductor. A potential is applied to the control grid of the same polarity as the corona potential but with a much lower voltage, usually several hundred volts, which suppresses the electric field between the charge plate and the corona wires and markedly reduces the ion current flow to the photoreceptor.

A recently developed corona charged device is described in U.S. Pat. No. 4,086,650 to Davis et al., commonly referred to in the art as a diconotron wherein the corona discharge electrode is coated with a relatively thick dielectric material such as glass so as to substantially prevent the flow of conduction current there-

through. The delivery of charge to the photoconductive surface is accomplished by means of a displacement current or capacitive coupling through the dielectric material. The flow of charge to the surface to be

5 charged is regulated by means of a DC bias applied to the corona shield. In operation an AC potential of from about 5,000 to 7,000 volts at a frequency of about 4 KHz produces a true corona current, an ion current of 1 to 2 millamps. This device has the advantage of providing a 10 uniform negative charge to the photoreceptor. In addition, it is a relatively low maintenance charging device in that it is the least sensitive of the charging devices to contamination by dirt and therefore does not have to be repeatedly cleaned.

15 In the diconotron device described above the dielectric coated corona discharge electrode is a coated wire supported between insulating end blocks and the device has a conductive auxiliary DC electrode positioned opposite to the imaging surface on which the charge is to be placed. In the conventional corona discharge device, the conductive corona electrode is also in the form of an elongated wire connected to a corona generating power supply and supported by end blocks with the wire being partially surrounded by a conductive shield which is usually electrically grounded. The surface to be charged is spaced from the wire on the side opposite the shield and is mounted on a conductive substrate.

20 In addition to the desirability to negatively charge one type of photoreceptor it often is desired to provide a negative precharge to another type photoreceptor such as a selenium alloy prior to its being actually positively charged. A negative precharging is used to neutralize the positive charge remaining on the photoreceptor after transfer of the developed toner image to the copy sheet and cleaning to prepare the photoreceptor for the next copying cycle. Typically in such a precharge corotron an AC potential of between 4,500 and 6,000 volts rms at 400 to 600 Hz may be applied. A 25 typical conventional corona discharge device of this type is shown generally in U.S. Pat. No. 2,836,725 in which a conductive corona electrode in the form of an elongated wire is connected to a corona generating AC voltage.

30 Certain difficulties have been observed when using corona charge devices that produce a negative corona. It is believed that various nitrogen oxide species are produced by the corona and that these nitrogen oxide species are adsorbed by solid surfaces. In particular it is believed that these oxide species are adsorbed by the conductive shield as well as the housing of the corona generating device. The shield may in principle be made from any conductor but is typically made from aluminum and the housing may be made from any of a number of structural plastics such as a glass filled polycarbonate. This adsorption of nitrogen oxide species occurs 35 despite the fact that during operation the corona generating device may be provided with a directed air flow to remove the nitrogen oxide species as well as to remove ozone. In fact during the process of collecting ozone the air flow may direct the nitrogen oxide species to an affected area of the charging device or even some other machine part. It has also been found that after such exposure when a machine is turned off for extended periods of idleness that the adsorbed nitrogen oxide species gradually are desorbed, that is the adsorption is 40 a physically reversible process. It should be understood 45 50 55 60 65

that the adsorbed and desorbed species are both nitrogenous but not necessarily the same, i.e., there may be conversion of  $\text{NO}_2$  to  $\text{HNO}_3$ . Then, when the operation of the machine is resumed, a copy quality defect is observed in the copies produced in that a line image deletion or lower density image is formed across the width of the photoreceptor at that portion of its surface which was at rest opposite the corona generating device during the period of idleness. While the mechanism of the interaction of the desorbed nitrogen oxide species and the photoreceptor layers is not fully understood, it is believed that they in some way interact with the surface of the photoreceptor increasing the lateral conductivity so that it cannot retain a charge in image fashion to be subsequently developed with toner. This basically causes narrow line images to blur or to wash out and not be developed as a toner image. This defect has been observed with conventional selenium photoreceptors which generally comprise a conductive drum substrate having a thin layer of selenium or alloy thereof vacuum deposited on its surface as the imaging surface. The difficulty is also perceived in photoreceptor configuration of plates, flexible belts, and the like, which may include one or more photoconductive layers in the supporting substrate. The supporting substrate may be conductive or may be coated with a conductive layer over which photoconductive layers may be coated. Alternatively, the multilayered electroconductive imaging photoreceptor may comprise at least two electrically operative layers, a photogenerating layer or a charge generating layer and a charge transport layer which are typically applied to the conductive layer. For further details of such a layer attention is directed to U.S. Pat. No. 4,265,990. In all these varying structures several of the layers may be applied with a vacuum deposition technique for very thin layers.

Furthermore, with prolonged exposure of the photoreceptor to the desorbing nitrogen oxide species during extended periods of idleness the severity of the line defect or line spreading increases. While the mechanism is not fully understood it has been observed that even after a relatively short period of time, 15 minutes, and a period of idleness of, say, several hours, a mild line defect and concurrent image deletion may be perceived. During the initial stage of exposure of the photoreceptor to the desorbing nitrogen oxide species, it is possible to rejuvenate the photoreceptor by washing with alcohol since reaction between the photoreceptor and the nitrogen oxide species is purely at the surface. However, after a prolonged period of time the reaction tends to penetrate the photoreceptor layer and cannot be washed off with the solvent. Thus, for example, the problem is perceived after a machine has been operated for about 10,000 copies, rested overnight and when the operator activates the machine the following morning, the line deletion defect will appear. As indicated above the defect is reversible to some degree by a rest period. However, the period involved may be of the order of several days which to an operator is objectionable.

Similar difficulties are encountered in a precharge corotron with a negative DC potential applied. Attempts to solve that problem by nickel plating the corotron shield met with limited success in that nickel combined with the nitrogen oxide species forming a nickel nitrate which is a deliquescent salt and on continued use becomes moist with water from the air eventually accumulating sufficient water that droplets may form and drop off onto the photoreceptor. Furthermore, the

nickel nitrate salts are green crystalline and loosely bonded rather than a cohesive durable film. In another attempt to solve a similar difficulty in a negative charging AC diconotron device the shield is coated first with a layer of nickel that is subsequently plated with gold. However, as a result of the extreme expense of gold, the gold is plated in a very thin layer and consequently the layer is discontinuous having numerous pores in the layer. Gold plating is theorized to provide a relatively inert surface which will not adsorb the nitrogen oxide species or will not permit conversion to a damaging form. However, with the thin porous layer of gold, the nickel substrate underneath the gold corrodes forming nickel nitrates in the same manner as with the precharge corotron and experiences similar difficulties resulting in limited useful life.

#### PRIOR ART

Item No. 19957 in the Research Disclosure Journal of November 1980 at page 508 describes an electrophotographic copying machine having corona charging unit wherein the ions generated from the corona discharge can interact with the photoconductive member and the conductive housing to form salts, e.g. nitrates which during an overnite period of rest may have a detrimental effect on the part of the stationary photoconductive member opposite the opening to the corona charging unit. This detrimental effect is claimed to be overcome by coating the inner side of the housing with a cellulose acetate butyrate copolymer in which carbon block particles have been dispersed.

U.S. Pat. No. 4,585,320 to Altavela et al. addresses this problem and provides a solution by means of plating the elements capable of adsorbing nitrogen oxide species with a thin layer of lead. U.S. Pat. No. 4,585,323 to Ewing et al. addresses the problem and teaches a remedy by providing a continuous thin layer of a paint containing a reactive metal such as nickel, lead, copper, silver and zinc on the surfaces which adsorbed the nitrogen oxide species. My U.S. Pat. No. 4,585,322 also addresses the problem and provides an alkali metal silicate coating on the elements capable of adsorbing and neutralizing the nitrogen oxide species.

In addition, my U.S. Pat. No. 4,646,196 also addresses the problem and provides a conductive dry film of aluminum hydroxide which may contain conductive particles such as graphite as a coating on the elements capable of absorbing and neutralizing the nitrogen oxide species. Electrodag 121 is disclosed as a coating.

While the coatings described in the above U.S. patents are capable to varying degrees of performing satisfactorily in certain applications certain difficulties are experienced. The most generally effective coatings in neutralizing corona effects have been the alkali metal silicate, particularly potassium silicate with graphite suspended in aqueous media as described in U.S. Pat. No. 4,585,322 and the aluminum hydroxide also with suspended graphite as described in U.S. Pat. No. 4,646,196. In particular, while the alkali metal silicate coatings when used as a coating on the conductive control grid of a scorotron charging device may be characterized as exhibiting long life in neutralizing the corona effects which lead to copy quality degradation they suffer from the difficulty that insulating particles form on the grid particularly at relatively low relative humidity. In particular, after about 8 hours use a white powder, presumably an alkali metal nitrate or carbonate is collected on the grid. The white powder on the grid

was found to alter the electrostatic relationship in the charging devices in that the current delivered to the control grid from the coronodes and the current delivered to the photoreceptor began to vary uncontrollably thereby providing an unpredictable, uneven charge on the photoreceptor, resulting in poor copy quality. The exact mechanism by which this happens is not fully understood, but is believed to be a combination of the holes becoming clogged with the white powder, the resistive nature of the coating, and the particulate nature of the nitrate powder. In particular, the ratio of the current to the control grid to the photoreceptor is determined generally by the geometry of the control grid, so if the holes are plugged, that geometry and the ratio of the current to the grid to the photoreceptor is altered. The resistive nature of the nitrate and carbonate powder causes it to change the effective bias on the grid by an amount equal to the voltage drop across the resistive powder layer. And finally, the particulate nature is believed to cause non-uniform electrical fields which in general tend to increase the current from the coronode.

On the other hand, the aluminum hydroxide suspensions described in U.S. Pat. No. 4,646,196 while they do not form contaminating insulating nitrate and carbonate salts on the scorotron grid exhibit an effluent neutralization life of only one tenth that of the potassium silicate based system.

#### SUMMARY OF THE INVENTION

In accordance with the present invention an improved corona generating device for depositing a negative charge on an imaging surface is provided wherein the damaging nitrogen oxide species generated by the corona charging unit and adsorbed by at least one element of the corona charging device adjacent the corona discharge electrode during operation and desorbed when at rest, are neutralized.

In accordance with the principle aspect of the present invention the element which adsorbs and desorbs the nitrogen oxide species is coated with a substantially continuous thin conductive dry film of aluminum hydroxide containing particulate graphite and powdered nickel to neutralize the nitrogen oxide species when they are generated.

In accordance with a further principle aspect of the invention said coating includes a binder, preferably a polyvinyl acetate binder, to provide adhesion of the film to the element and cohesion within the film matrix.

In a further principle aspect of the present invention, the element which adsorbs and desorbs the nitrogen oxide species comprises a conductive corona control grid of a scorotron charging device.

In a further aspect of the present invention the grid is made from a beryllium copper alloy preferably containing from about 0.1% to 2.0% by weight beryllium.

In a further aspect of the present invention the aluminum hydroxide film exists as the unhydrated oxide, a hydrated oxide, aluminum hydroxide or mixtures thereof.

In a further aspect of the present invention, the element which adsorbs and desorbs the nitrogen oxide species comprises a conductive shield which substantially surrounds the corona discharge electrode and has a longitudinal opening therein to permit ions emitted from the electrode to be directed toward the surface to be charged.

In a further aspect of the present invention, the corona discharge electrode comprises a thin wire coated at least in the discharge area with a dielectric material.

In a further aspect of the present invention, the corona generating device comprises a planar shield and includes an insulating housing having two sides adjacent such shield to define a longitudinal opening to permit ions emitted from the electrode to be directed toward the surface to be charged. The two sides of the insulating housing as well as a conductive shield are coated with a substantially continuous thin conductive dry film of aluminum hydroxide containing graphite particles and powdered nickel.

In a further aspect of the present invention the film is from about 0.3 to about 1.0 mil in thickness.

For a better understanding of the invention as well as other aspects and further features thereof, reference is had to the following drawings and descriptions.

#### BRIEF DESCRIPTION OF THE DRAWINGS

FIG. 1 is an illustrative cross section of a corona discharge device according to the present invention.

FIG. 2 is an isometric view of a preferred embodiment of a diconotron according to the present invention.

FIG. 3 is an isometric view of another preferred embodiment of a corotron according to the present invention.

FIG. 4 is an isometric view of another preferred embodiment of a scorotron according to the present invention.

FIG. 5 is an enlarged view of the control grid used in the scorotron illustrated in FIG. 4.

#### DESCRIPTION OF THE PREFERRED EMBODIMENTS

Referring to FIG. 1 the corona generator 10 of this invention is seen to comprise a corona discharge electrode 11 in the form of a conductive wire 12 having a relatively thick coating 13 of dielectric material.

A charge collecting surface 14 is shown which may be a photoconductive surface in a conventional xerographic systems. The charge collecting surface 14 is carried on a conductive substrate 15 held at a reference potential, usually machine ground. An AC voltage source 18 is connected between the substrate 15 and the corona wire 12, the magnitude of the AC source being selected to generate a corona discharge adjacent the wire 12. A conductive shield 20 is located adjacent the corona wire on the side of the wire opposite the chargeable surface.

The shield 20 has coupled thereto a switch 22 which depending on its position, permits the corona device to be operated in either a charge neutralizing mode or a charge deposition mode. With the switch 22 as shown, the shield 20 of the corona device is coupled to ground via a lead 24. In this position, no DC field is generated between the surface 14 and the shield 15 and the corona device operates to neutralize over a number of AC cycles any charge present on the surface 14.

With switch 22 in either of the positions shown by dotted lines, the shield is coupled to one terminal of a DC source 23 or 27, the other terminals of the sources being coupled by lead 26 to ground thereby establish a DC field between the surface 14 and the shield 20. In this position, the corona operates to deposit a net charge onto the surface 14, the polarity and magnitude of this charge depends on the polarity and magnitude of the DC bias applied to the shield 20.

The corona wire 13 may be supported in conventional fashion at the ends thereof by insulating end blocks (not shown) mounted within the ends of shield structure 20. The wire 12 may be made of any conventional conductive filament material such as stainless steel, gold, aluminum, copper, tungsten, platinum or the like. The diameter of the wire 11 is not critical and may vary typically between 0.5-15 mils and preferably is about 9 mils.

Any suitable dielectric material may be employed as the coating 13 which will not break down under the applied corona AC voltage, and which will withstand chemical attack under the conditions present in a corona device. Inorganic dielectrics have been found to perform more satisfactorily than organic dielectrics due to their higher voltage breakdown properties, and greater resistance to chemical reaction in the corona environment.

The thickness of the dielectric coating 13 used in the corona device of the invention is such that substantially no conduction current or DC charging current is permitted therethrough. Typically, the thickness is such that the combined wire and dielectric thickness falls in the range from 7-30 mil with typically dielectric thickness of 2-10 mil. Glasses with dielectric breakdown strengths above 2 KV/mil at 4 KHz and in the range of 2 to 5 mil thickness have been found by experiment to perform satisfactorily as the dielectric coating material. As the frequency or thickness go down the strength in volts per mil will usually increase. The glass coating selected should be free of voids and inclusions and make good contact with or wet the wire on which it is deposited. Other possible coatings are ceramic materials such as alumina, zirconia, boron nitride, beryllium oxide and silicon nitride. Organic dielectrics which are sufficiently stable in corona may also be used.

The frequency of the AC source 18 may be varied widely in the range from 60 Hz commercial source to several megahertz. The device has been operated and tested at 4 KHz and found to operate satisfactorily.

The shield 20 is shown as being semi-circular in shape but any of the conventional shapes used for corona shields in xerographic charging may be employed. In fact, the function of the shield 20 may be performed by any conductive member, for example, a bare wire, in the vicinity of the wire, the precise location not being critical in order to obtain satisfactory operation of the device.

With the switch 22 connected as shown so that the shield 20 is grounded, the device operates to inherently neutralize any charge present on the surface 14. This is a result of the fact that no net DC charging current passes through the electrode 11 by virtue of the thick dielectric coating 13 and the wire 12.

Referring to FIG. 1, operation of the corona device of the invention to deposit a specific net charge on an imaging surface is accomplished by moving switch 22 to one of the positions shown in dotted lines, whereby a DC potential of either positive polarity or negative polarity with respect to the surface 15 may be applied to the shield.

In charging operation typical AC voltages applied to the corona electrodes are in the range from 4 KV to 7 KV at a frequency between 1 KHz and 10 KHz. With the conductive substrate of the imaging member being held at ground potential a negative DC bias of from about 800 volts to about 4 KV is applied to the shield. For further details of the manner of operation of the

above described dicorotron device, attention is directed to U.S. Pat. No. 4,086,650 to Davis et al.

Referring once again to FIG. 1, the shield 20 is coated at least on its top with a substantially continuous thin conductive dry film 28 of aluminum hydroxide containing graphite particles and powdered nickel to neutralize the nitrogen oxide species that may be generated when a dicorotron is energized. Typically the dry film is formed by drying or dehydrating a liquid dispersion; 10 preferably aqueous, which has been applied as a somewhat gelatinous coating to the substrate shield. Typically, the graphite is present in the dispersion in an amount from about 7 percent to 13 percent by weight of the total weight of the dispersion. The graphite particles 15 are typically from about 0.04 micrometers to about 22 micrometers in size. The powdered nickel is present in the dispersion in an amount of from about 3 percent to about 5 percent by weight of the total weight of the dispersion. Typically, the nickel powders have a particle size of from about 1.1 micrometers to about 34 micrometers. In addition, small quantities up to about 10% by weight of the total weight of the film of non-reactive 20 filler such as silica may be present in the coating composition. It is believed that such nonreactive filler provides film resilience to the corona environment. Reactive conductive fillers such as metallic particles are not preferred since they tend to react with the nitrogen oxide species forming nitrate powders.

While such a composition is capable of performing satisfactorily it is preferred to include a binder in the coating composition to enhance the mechanical properties of the film such as its adhesion to the substrate to be coated and the cohesion of the dried film matrix. Typically, the binders are water soluble and dispersible resins which are present in amounts up to about 34 percent by weight of the total weight of the dry conductive film. Polyvinyl acetate is a typical such binder

The substantially continuous thin conductive dry film of aluminum hydroxide containing graphite particles 40 and powdered nickel may be formed on the surface to be coated by applying an aqueous solution or dispersion as a thin film thereto. Typically the dry films can be formed by applying the coating dispersion by spraying, including electrostatic spraying, or brushing as with a paint or by dip coating. Upon drying which includes room and elevated temperature the liquid films dehydrate so as to provide a coherent film with a strong rigid adhesive bond to the surface to be coated. The dispersion is applied in a thickness that will not be consumed in a reasonable period of time by the irreversible neutralization of the nitrogen oxides. Typically, it is applied in a thickness to provide a dry film thickness of from about 0.3 to about 1.0 mil as a substantially uniform continuous layer without pores. The film may be applied in a single layer or in multiple layers as desired. The exact mechanism by which the aluminum hydroxide film containing graphite and nickel provides long effective life in neutralizing the nitrogen oxides species without the formation and buildup of nitrate and carbonate salts is not understood. However, it is believed that the aluminum hydroxide combines with the nitrogen oxide species to form an aluminum nitrate in an irreversible reaction but no white powder is observed. Such a mechanism would completely remove the possibility of exposure of the photoreceptor to the nitrogen oxide species. Since no white powder is observed it is believed that the reaction may take place slowly on a molecular scale which is not perceived by the unaided

eye with the reaction products remaining dispersed in the original film. Furthermore, the adherent film formed on drying is believed to exist as the unhydrated aluminum oxide, a hydrated oxide or aluminum hydroxide or mixtures thereof. One way of characterizing the action of the aluminum oxide-hydrated is as an aluminum hydroxide which in the presence of nitrogen oxides acts as a base according to the following net reaction:



The nickel powder in the film also tends to neutralize the nitrogen oxide species, however, this occurs with substantially no salt formation. In this regard nickel powder is somewhat unique. The presence of the nickel powder also enhances the conductivity imparted to the film by the presence of the graphite particles.

FIG. 2 illustrates a preferred embodiment in the diconotron device according to the present invention. In FIG. 2 the diconotron wire 30 is supported between anchors 31 at opposite ends which are anchored in end blocks 35. The conductive shield 34 is constructed in tubular fashion in such a way as to be slideably mounted in the bottom of the housing 39 by means of handle 36. The shield is connected to the power supply through a sliding contact on its inner surface to a leaf spring which in turn is connected to a DC pin connector (not shown). The power supply potential may be positive, negative, or zero (grounded) depending on device function. It is fastened in place when inserted within the housing 39 by means of spring retaining member 38. When inserted in the machine high voltage contact pin 33 provides the necessary contact to the AC power supply. In addition to the conductive shield 34 the housing 39 comprises two vertically extending side panels 32 extending the entire length of the diconotron wire. Both the top and inner surfaces of the shield 34 may have a substantially continuous thin conductive dry film of aluminum hydroxide containing graphite and nickel powder. In addition, the vertically extending panels 32 of the housing 39 may also be coated with a film 40 according to the present invention. The housing 39 together with the side panels 32 may be made from a single one piece molding from any suitable material such as glass filled polycarbonate.

FIGS. 4 and 5 illustrate alternative preferred embodiments according to the present invention which embody use of the present invention in coating the conductive corona control grid of a scorotron. In FIG. 4, scorotron 57 is represented as including two linear pin electrode arrays 58, and 59 supported between insulating end block assemblies 61 and 62. The conductive corona control grid 64 is placed on top of the linear pin arrays and anchored in place by means of screw 65 to potential generating source by lead 66. Both of the linear pin electrode arrays 58 and 59 are connected to potential generating source 67. Such a device might have utility as a negative charging corona generating device wherein the potential from a high voltage DC power supply applied to the grid is about -800 volts or very close to the voltage desired on the imaging surface which is closely spaced therefrom. The potential applied to the two linear pin electrode arrays is in the range of from about -6,000 to about -8,000 volts. The entire assembly is supported by being clamped between three injection molded plastic support strips. In this configuration the two linear pin coronodes in the shape of a saw tooth provide vertically directional fields and

currents due to their geometry providing a higher efficiency of current to the photoconductor versus the total current generated. The grid acts as a leveling device or reference potential limiting the potential on the substrate being charged. In accordance with the present invention, the grid may be coated with a substantially continuous thin conductive dry film of aluminum hydroxide containing graphite and powdered nickel. In a preferred embodiment of the present invention the grid is fabricated from a beryllium copper alloy since it appears to reduce the effect of the nitrogen oxide species when compared to other metals such as stainless steel. Typically, beryllium is present in the alloy in an amount of from about 0.1% to about 2.0% by weight. A preferred alloy is Copper Development Associates 172 (CDA 172) which is 1.8% by weight beryllium. In a particularly preferred embodiment the pin electrodes are also made of the same beryllium copper alloys.

The efficiency of several different coatings was evaluated using a pin scorotron array and grid as illustrated in FIGS. 4 and 5 for both a grid made from stainless steel and one made from beryllium copper alloy.

In the tests, the scorotron screens or grids were driven in a test fixture at common voltage levels of -1000 volts. Voltage was applied to the coronode to produce a 2 milliamp corona current. Testing was performed in a high humidity environment, conducive to the production of deletions. The screen was spaced 0.118 in (3 mm) from a bare aluminum surface. The screens were coated with the selected coatings, as described. Periodically, about every 48 hours, the scorotrons were removed from the aging fixture, the pins cleaned, and the scorotrons inserted into a Xerox 1065 copier to produce copies for evaluation. The scorotrons were allowed to "outgas" or desorb nitrogen oxide species for 20 minutes. Several copies of a test pattern were made and the parking deletion level was scored by the following convention:

|          |                                                                                                                                                                                         |
|----------|-----------------------------------------------------------------------------------------------------------------------------------------------------------------------------------------|
| level 0: | No deletion visible on any copies.                                                                                                                                                      |
| level 1: | Slight lightening of image<br>Small in size: <3 in (76.3 mm) long $\times$ <1 in (25.4 mm) wide.                                                                                        |
| level 2: | Moderate lightening of image<br>Moderate in size: <6 in (152.4 mm) long $\times$ <1 in (25.4 mm) wide.                                                                                  |
| level 3: | Moderate lightening of image at edges with center of defect slightly darkened to near original image density.<br>Moderate in size: <6 in (152.4 mm) long $\times$ <1 in (25.4 mm) wide. |
| level 4: | Lightening of image at edges with center of defect noticeably darkened.<br>Large size: >6 in (152.4 mm) long $\times$ >1 in (25.4 mm) wide.                                             |
| level 5: | Loss of image at edges with center of defect very dark.<br>Large size: >6 in (152.4 mm) long $\times$ >1 in (25.4 mm) wide.                                                             |

In the above-defined measurement scale, a level 3 deletion would be satisfactory for most copying or printing applications involving print images, but would be somewhat less than satisfactory for pictorial or graphic images. In some applications a level 1 deletion would be unsatisfactory.

Subsequent to each production of test documents, the scorotrons were returned to the test fixture. The tests were made over a period of 500 hours. The parking deletion/time track performance are tabulated for the

following examples. In the examples all parts and percentages are by weight unless otherwise stated. Examples 1a, 1b are for comparison purposes only.

### EXAMPLES 1a, 1b

Screens are coated with an Electrodag 121 as described in my U.S. Pat. No. 4,646,196. Electrodag 121, available from Acheson Colloid Company, Port Huron, Mich., is an aqueous dispersion of semicolloidal graphite in an inorganic binder which cures at 350° C. in one hour to form a hard conductive coating, and which is believed to contain by weight, 77.5% water, 14.5% aluminum oxide hydrated, 7% graphite and about 1% polyvinylpyrrolidone. Both sides of the screens were sprayed with the composition and the screens permitted to dry prior to being placed in the test fixture. Example 1b is a beryllium copper screen and 1a is a 304 Stainless Steel Screen. The results of the test are tabulated in TABLE 1.

TABLE 1

| Time (hrs) | Example 1a<br>Deletion Level<br>of Example 1a<br>on 304SST | Example 1b<br>Deletion Level<br>of Example 1b<br>on BeCu |
|------------|------------------------------------------------------------|----------------------------------------------------------|
| 0          | 0                                                          | 0                                                        |
| 41         | 0                                                          | 0                                                        |
| 83         | 2                                                          | 0                                                        |
| 138        | 4                                                          | 0                                                        |
| 188        | 3                                                          | 1                                                        |
| 260        | 4                                                          | 2                                                        |
| 346        | 4                                                          | 3                                                        |
| 418        | 5                                                          | 3                                                        |
| 500        | 5                                                          | 4                                                        |

### EXAMPLES 2a, 2b

The procedure of Examples 1 is repeated except that the coating composition includes powdered nickel and is believed to have about 21% solids content containing by weight about 14.5% aluminum oxide hydrated, 36% graphite, 36% nickel, and 8.5% silica.

The results of testing a stainless steel screen, Example 2a, and a beryllium copper screen, Example 2b, are tabulated in TABLE 2.

TABLE 2

| Time (hrs) | Example 2a<br>Deletion<br>Level of<br>Example 2a<br>on 304 SST | Example 2b<br>Deletion<br>Level of<br>Example 2b<br>on BeCu |
|------------|----------------------------------------------------------------|-------------------------------------------------------------|
| 0          | 0                                                              | 0                                                           |
| 41         | 0                                                              | 0                                                           |
| 83         | 0                                                              | 0                                                           |
| 138        | 1                                                              | 0                                                           |
| 188        | 3                                                              | 0                                                           |
| 260        | 4                                                              | 0                                                           |
| 346        | 5                                                              | 0                                                           |
| 418        | 5                                                              | 0                                                           |
| 500        | 5                                                              | 0                                                           |

### EXAMPLES 3a, 3b

The procedure of Examples 2a and 2b is repeated except that the solids content of the coating composition is believed to have about 54% by weight graphite and 18% by weight nickel. The results of testing a stainless steel screen, Example 3a, and a beryllium copper screen, Example 3b, are tabulated in TABLE 3.

TABLE 3

| Time (hrs) | Example 3a<br>Deletion<br>Level of<br>Example 3a<br>on 304 SST | Example 3b<br>Deletion<br>Level of<br>Example 3b<br>on BeCu |
|------------|----------------------------------------------------------------|-------------------------------------------------------------|
| 0          | 0                                                              | 0                                                           |
| 41         | 0                                                              | 0                                                           |
| 83         | 1                                                              | 0                                                           |
| 138        | 5                                                              | 0                                                           |
| 188        | 4                                                              | 0                                                           |
| 260        | 4                                                              | 0                                                           |
| 346        | 5                                                              | 0                                                           |
| 418        | 5                                                              | 0                                                           |
| 500        | 5                                                              | 1                                                           |

### EXAMPLES 4-6

The procedure of Example 1 is repeated except that all the screens evaluated were beryllium copper alloy 172 BeCu and three different coating compositions as follows were evaluated at about 75, 125, 175, 225, 300, 350 and 400 hours.

### EXAMPLE 4

25 The beryllium copper screen was plated with nickel metal to a thickness of about 0.5 mils.

### EXAMPLE 5

30 The beryllium copper screen was coated with the composition of Examples 1a and 1b.

### EXAMPLE 6

35 The beryllium copper screen was coated with a composition believed to have about a 25.5% by weight solids content containing about 10% aluminum oxide hydrated, 35% graphite, 15% nickel and 5.5% silica and 30.5% of a polyvinyl acetate modified by a low level hydrolysis process to form a polyvinyl alcohol comonomer to promote adhesion.

40 The test results are tabulated in TABLE 4.

TABLE 4

| Time (hrs) | Deletion<br>Level<br>Example 4 | Deletion<br>Level<br>Example 5 | Deletion<br>Level<br>Example 6 |
|------------|--------------------------------|--------------------------------|--------------------------------|
| 75         | 0                              | 0                              | 0                              |
| 125        | 1                              | 1                              | 0                              |
| 175        | 1                              | 1                              | 0                              |
| 225        | 1                              | 3                              | 0                              |
| 300        | 2                              | 2                              | 0                              |
| 350        | 1                              | 2                              | 0                              |
| 400        | 1                              | 0                              | 0                              |

55 Comparison between comparative Examples 1a, 1b, 4 and 5 with Examples according to the invention 2a, 2b, 3a, 3b, and 6 reveals the improved functional life achieved according to the practice of the present invention. While comparison of Example 2a with 1a shows only somewhat modest improvement in deletion level with the stainless steel screen the improved performance of the coating composition according to the invention is dramatically demonstrated in comparing Example 2b with 2a noting that there is no reduction in deletion level over 500 hours when used with the beryllium copper substrate. Similarly, when comparing Example 3b with 1b wherein 500 hours has elapsed before deletion level 1 is experienced. It is noted with reference to Example 3a that the results are believed to be due to an adhesion failure in the dry film on the stainless

steel substrate. Example 6 shows a superior performance is also achieved when an adhesion and cohesion promoting binder is added. Thus, a significant useful life extension is believed to be realized when using the composition according to the present invention on charging devices to neutralize nitrogen oxide species formed during the charging operation. The charging devices of the present invention having a highly corrosion resistant, water resistant, adherent coating which does not result in the formation of excessive insulating nitrate 10 deposits which inhibit the function of the charging device. In a the preferred embodiment wherein a beryllium copper alloy is used, while not wishing to be bound to any particular theory it is believed that the coating according to the present invention functions to prevent oxidation of the beryllium copper alloy thereby avoiding the formation of an oxide barrier layer which inhibits the neutralizing effect of the beryllium copper alloy on the nitrogen oxide species.

All the patents and the article referred to herein are 20 hereby incorporated by reference in their entirety to the instant specification.

While the invention has been described with reference to the specific embodiments it will be apparent to those skilled in the art that many alternatives, modifications and variations may be made. It is intended to embrace such modifications and alternatives as may fall within the spirit and scope of the appended claims.

I claim:

1. A corona generating device for depositing a negative charge on an imaging surface carried on a conductive substrate held at a reference potential comprising; at least one elongated conductive corona discharge electrode supported between insulating end blocks, means to connect said electrode to a corona generating potential source, at least one element adjacent said corona discharge electrode capable of adsorbing nitrogen oxide species generated when said corona discharge electrode is energized and capable of desorbing nitrogen oxide species when said electrode is not energized, said at least one element being coated with a substantially continuous thin conductive dry film of aluminum hydroxide containing graphite and powdered nickel, said film having been formed from a liquid dispersion of aluminum hydroxide containing from about 7 to about 13 percent by weight graphite and from about 3 percent to about 10 percent by weight nickel by weight of the total weight of the dispersion.
2. The corona generating device of claim 1, further comprising a binder to provide adhesion of said film to said element and cohesion within the matrix of said film.
3. The corona generating device of claim 2, wherein said binder is a polyvinyl acetate binder.

4. The corona generating device of claim 1, wherein said film is from 0.3 to about 1.0 mil in thickness.

5. The corona generating device of claim 1, wherein the aluminum hydroxide film exists as the unhydrated oxide, a hydrated oxide, aluminum hydroxide or mixtures thereof.

6. The corona generating device of claim 1, wherein said at least one elongated conductive corona discharge electrode comprises at least one linear array of pin electrodes.

7. The corona generating device of claim 1, wherein said at least one element comprises a conductive corona control grid.

8. The corona generating device of claim 7, wherein said grid is made from a beryllium copper alloy.

9. The corona generating device of claim 8, wherein said beryllium copper alloy comprises from about 0.1% to about 2.0% by weight beryllium.

10. The corona generating device of claim 2, wherein said at least one elongated conductive corona discharge electrode comprises at least one linear array of pin electrodes.

11. The corona generating device of claim 10, wherein said at least one element comprises a conductive corona control grid.

12. The corona generating device of claim 11, wherein said grid is made from a beryllium copper alloy.

13. The corona generating device of claim 12, wherein said beryllium copper alloy comprises from about 0.1% to about 2.0% by weight beryllium.

14. The corona generating device of claim 1, wherein said at least one element comprises a conductive shield which substantially surrounds said corona discharge electrode and has a longitudinal opening therein to permit ions emitted from the electrode to be directed toward the surface to be charged.

15. The corona generating device of claim 14, wherein said corona discharge electrode comprises a thin wire coated at least in the discharge area with a dielectric material, and said conductive shield has means associated therewith to connect to a potential source.

16. The corona generating device of claim 14, wherein said shield is planar on one side of the corona discharge electrode and further including an insulating housing having two sides adjacent said shield to define a longitudinal opening to permit ions emitted from the electrode to be directed toward a surface to be charged, said two sides of said insulating housing being coated with a substantially continuous thin conductive dry film of aluminum hydroxide.

17. The corona generating device of claim 15, wherein said dielectric material is glass.

\* \* \* \* \*